

## UNITED STATES PATENT OFFICE

2,181,936

## ROLLING OF CATHODE NICKEL

Robert R. Clappier, Huntington, W. Va., and James Orin McDowell, Steubenville, Ohio, assignors to The International Nickel Company, Inc., New York, N. Y., a corporation of Delaware

No Drawing. Application February 4, 1938,  
Serial No. 188,630

## 2 Claims. (Cl. 29—18)

The present invention relates to a rolling process for producing nickel strip of uniform gauge and shape directly from nickel cathodes.

In the past many attempts have been made to cold roll nickel cathodes to uniform gauge and shape without pre-treatment. As far as we are aware such attempts have not been wholly successful when carried into practise on a commercial scale. These attempts may have failed from various causes among which has been the variation in gauge of an individual cathode. Such variations in gauge made it practically impossible to cold roll nickel cathode directly to strip of uniform gauge and shape. It is obvious that the gauge of the cathode could be controlled during electro-deposition of the nickel but such control of conditions in the plating tank would necessitate seriously curtailing the output of the plating tanks. Direct cold rolling of cathode nickel of variable thickness resulted in the production of strip of non-uniform shape and gauge.

It is possible to use cathode nickel for strips by melting, refining, pouring into ingots and forging, but this solution of the problem is time consuming and increases the cost of production exceedingly.

We have discovered a process of dispensing with all of the conventional steps of melting, pouring and forging, etc., and of rolling cathode nickel directly into strip of uniform shape and gauge.

It is an object of the present invention to provide a process of rolling cathode nickel directly into strip of uniform shape and gauge on an industrial scale.

It is another object of the present invention to eliminate the necessity of customary melting, pouring, forging, etc., of cathode nickel preparatory to producing nickel strip of uniform shape and gauge.

It is a further object of the present invention to provide a substantially direct cold rolling process for producing nickel strip of uniform shape and gauge from cathode nickel involving the use of a special hot rolling pre-treatment.

Other objects and advantages will become apparent from the following description of a preferred embodiment of the invention.

In general, the process according to the present invention contemplates the heating of the cathode of varying gauge to a hot rolling temperature and then subjecting it to a special hot rolling pretreatment by giving the cathode a single heavy pass on a hot mill, or, if desired, it may be given two or more lighter passes. After the preliminary pass or passes on the hot mill, the

partially rolled strip is finished on the cold mill.

For the purpose of giving those skilled in the art a better understanding, the following illustrative example is given.

A nickel cathode about 33 $\frac{1}{2}$  inches in width, about 26 $\frac{1}{2}$  inches in length and having an average thickness of about 0.250 inch but varying in gauge from about .229 inch to about .279 inch was heated to a temperature of about 1900° F. to about 2000° F. and passed through a hot mill of conventional design with 2 to 4 passes giving about 50% reduction in cross section. The partially rolled sheet had the following dimensions: about 49 inches in length and about 34 $\frac{1}{2}$  inches in width and was of uniform shape with the gauge varying between about .135 inch and about .139 inch. From the hot mill, the strip was passed through a cold mill and given successive reductions of about 1% to about 5% per pass and about 60% total reduction in cross section. Finishing cold passes were less than about 1 per cent reduction. The resulting step had a gauge of about 0.058 of an inch plus or minus about 0.001 of an inch. The finished sheet is about 35 inches in width and about 116 inches in length and the gauge of the finished strip is uniform to within about 0.002 of an inch.

As those skilled in the art are aware, commercial nickel cathodes, as they come from tanks operated on an industrial scale, do not have a smooth surface. On the contrary, there are numerous surface imperfections which give it a somewhat warty appearance. These warty growths are commonly called "berries". The special hot rolling pretreatment of such cathodes, in accordance with the principles of the present invention, smooths out these "berries", so that the partially rolled sheet which passes from the hot mill to the cold mill has a practically smooth surface. In consequence of the novel combination of operations involved in the present invention, cold rolled sheet and strip nickel are produced from commercial non-uniform nickel cathodes under industrial conditions and on standard mill equipment which sheet and strip possess satisfactory and acceptable uniformity of gauge and shape. This new result is of great commercial importance because of the economies it effects over the conventional practice of melting, refining, pouring into ingots, forging, rolling, etc.

We claim:

1. A process for producing nickel strip having a smooth surface and substantially uniform gauge and shape in widths as high as about 35 inches

directly from a nickel cathode having a rough surface on which are numerous berries and non-uniform gauge comprising heating the cathode to a temperature between about 1900° F. and 5 2000° F., passing the heated cathode about 2 to 4 times through a hot rolling mill to reduce its cross section about 50% and thereby practically to smooth out the berries and gauge inequalities and passing the cathode through a cold mill with 10 successive reductions of about 1% to 5% per pass to further reduce the cross section about 60% and thereby completely to smooth out the berries and gauge inequalities, whereby nickel strip having a smooth surface and substantially uniform gauge 15 and shape in widths as high as about 35 inches is produced.

2. A process for producing nickel strip having a smooth surface and substantially uniform gauge

and shape in widths as high as about 35 inches directly from a nickel cathode having a rough surface on which are numerous berries and non-uniform gauge comprising heating the cathode to a hot rolling temperature, passing the cathode 5 through a hot mill to reduce the cross section substantially in heavy passes and thereby practically to smooth out the berries and gauge inequalities, and passing the cathode through a cold mill with successive light reductions to further reduce the cross section substantially and thereby completely to smooth out the berries and gauge inequalities, whereby nickel strip having a smooth surface and substantially uniform gauge and shape in widths as high as about 35 inches 10 is produced.

ROBERT R. CLAPPIER.  
JAMES ORIN McDOWELL.

CERTIFICATE OF CORRECTION.

Patent No. 2,181,936.

December 5, 1939.

ROBERT R. CLAPPIER, ET AL.

It is hereby certified that error appears in the printed specification of the above numbered patent requiring correction as follows: Page 1, second column, line 22, for the word "step" read strip; and that the said Letters Patent should be read with this correction therein that the same may conform to the record of the case in the Patent Office.

Signed and sealed this 6th day of February, A. D. 1940.

(Seal)

Henry Van Arsdale,  
Acting Commissioner of Patents.